

# United States Patent Office

3,296,139

Patented Jan. 3, 1967

1

3.296.139

3,296,139

**ORGANIC PEROXY ESTER ANTI-SEIZURE AGENT**  
Arthur M. Shapiro, Philadelphia, Pa., assignor to the  
United States of America as represented by the Secre-  
tary of the Army  
No Drawing. Filed Mar. 4, 1965, Ser. No. 437,323  
5 Claims. (Cl. 252—57)

The invention described herein may be manufactured and used by or for the Government for governmental purposes without the payment to me of any royalty thereon.

This invention relates to improved lubricants containing as a major lubricating component oil of mineral origin. In particular, the invention relates to lubricating compositions of this type having improved anti-seizure and anti-wear characteristics.

A particular property required by many mineral base lubricants used today is an ability to prevent seizure and scoring of relatively moving metallic surfaces operating under extremely high pressures per unit area, in many cases considerably in excess of 10,000 p.s.i. Pressures on this order have long been encountered in the machine industry and in metal machining operations which undergo extremely high pressure loads. Consequently, for effective lubrication, lubricants capable of withstanding pressures appreciably higher than those at which ordinary mineral base oil lubricant films will rupture have been required.

It is therefore a principal object of the invention to provide a compounded lubricating product of mineral base oil possessing good anti-seizure and anti-wear characteristics of a high order as those encountered in high speed cutting of metals and in other diverse machine operations where high pressures are present.

It is another object of the invention to provide a lubricant having improved anti-seizure and anti-wear properties, said lubricant comprising a major proportion of an oil of mineral origin having an organic peroxy ester blended therewith.

Other objects and features of the invention will become apparent as the invention is more fully hereinafter disclosed.

In accordance with these objects it has been discovered that minor additions of an organic peroxy ester to mineral based oils are characterized by good anti-seizure and anti-wear properties. More specifically, I have found that *t*-butyl perbenzoate is capable of imparting these desirable properties to mineral base oils.

Mineral oil SAE 10 only is presented in the table following. It is to be understood however that the invention is not to be considered as being limited to this specific viscosity as it will be apparent to those skilled in the art that a wide variety of viscosities of mineral oils may be employed in formulating the lubricant contemplated herein.

The lubricity agent of my present invention is available commercially, 0.5 through 3.0 weight percentages of t-butyl perbenzoate, having an empirical formula of  $C_{11}H_{14}O_3$ , a molecular weight of 194.2 and a structural formula of



was intimately blended with varying SAE mineral oils and then subjected to anti-seizure and anti-wear evaluation tests. These tests were conducted on conventional laboratory equipment and will not be described, their operations being well known to those skilled in the art. For example, anti-wear data were obtained on the Shell

2

4-ball wear tester while anti-seizure data were determined using the well known Falex extreme pressure tester. Description of the Shell 4-ball tester may be found in an article by G. D. Boerlage, Engineering, vol. 136 (1933), p. 46 et seq. The Falex extreme pressure tester is described in Lubrication Engineering, September 1946, V. A. Ryan.

The tabulated comparative data following illustrates the extreme pressure or anti-seizure and anti-wear effectiveness of the present invention when incorporated in a mineral base oil such as SAE 10.

| Additive            | Wt.<br>Percent<br>Additive | Shell 4-Ball<br>Wear Scar<br>Diameter<br>(mm.) | Falex Extreme<br>Pressure Jaw<br>Load at<br>Failure (lbs.) |
|---------------------|----------------------------|------------------------------------------------|------------------------------------------------------------|
| None                |                            | 0.72                                           | 250                                                        |
| t-Butyl Perbenzoate | 0.5                        | 0.51                                           | 1,000                                                      |
| Do                  | 1.0                        | 0.45                                           | 1,250                                                      |
| Do                  | 2.0                        | 0.37                                           | 2,500                                                      |
| Do                  | 3.0                        | 0.35                                           | 3,500                                                      |

The wear tests were conducted on standard 52100 steel whereas the extreme pressure tests were conducted with blocks of C1144 steel and a pin of SAE 8640 steel. In addition to the property of being able to withstand high anti-seizure loads and wear there are other factors which must be considered in evaluating a lubricant. Among the most important is the tendency of the lubricant to corrode the containers in which it is stored and the metals with which it comes in contact during use. The above tabulated data show my t-butyl perbenzoate to impart excellent anti-seizure and anti-wear properties to steel machining operations. Commercial cutting oils normally contain phosphorous, chlorine and sulfur type additives, the latter two being the most corrosive.

It should be apparent therefor that the lubricant of my present invention, being devoid of these harmful elements will not tend to corrode the metals as greatly as commercial cutting oils.

All values presented in the table are averages of five different measurements. Maximum variance among the five values was confined to within a 10% range. Although 0.5 to 3.0 weight percentages of the lubricity additive of my invention is presented only, it should be understood that intermediate additions were found equally satisfactory, that is, between 0.5 and 3.0 weight percentages.

50 From the data hereinabove set forth, it will become evident that the lubricity additive of the present invention, when confined within the prescribed range, improves both anti-seizure and anti-wear characteristics of the mineral base oil. Further, its corrosive tendencies are 55 considerably lower than the presently used commercial cutting oils. Amounts of my respective lubricity additive below about 0.5 weight percent do not produce sufficient advantageous effects to render the composite oil lubricant adequate for anti-seizure and anti-wear use. Similarly, 60 if the additive is incorporated with the mineral oil in quantities greater than about 3 weight percent, the composite lubricant shows little further improvement in the level of these properties and, in several instances, a slight decrease in levels results.

65 I claim:

70 1. A lubricant composition having good anti-seizure, anti-wear and anti-corrosive properties suitable for use in various machine cutting operations, said lubricant composition consisting essentially of about 0.5 to 3.0 weight percent of t-butyl perbenzoate and the balance being an oil of mineral origin.

2. A lubricant according to claim 1 wherein said t-butyl perbenzoate is present in an amount of about 0.5 weight percent.
3. A lubricant according to claim 1 wherein said t-butyl perbenzoate is present in an amount of about 1.0 weight percent.
4. A lubricant according to claim 1 wherein said t-butyl perbenzoate is present in an amount of about 2.0 weight percent.
5. A lubricant according to claim 1 wherein said t-butyl perbenzoate is present in an amount of 3.0 weight percent.

## References Cited by the Examiner

## UNITED STATES PATENTS

1,766,501 6/1930 Buerk 44-57

## OTHER REFERENCES

Sato et al.: "Chemical Abstracts," page 7941, volume 53 (1959), "Effect of Peroxides on the Rust Preventing Properties of Oils."

10 DANIEL E. WYMAN, Primary Examiner.  
W. H. CANNON, Assistant Examiner.